

# United States Patent Office

3,024,195

Patented Mar. 6, 1962

1

3.024.195

**LUBRICATING OIL COMPOSITIONS OF ALKYL-  
PIPERAZINE ALKENYL SUCCINIMIDES**

ALAN Y. DRUMMOND, Richmond, Robert G. Anderson, Novato, and Frank A. Stuart, Orinda, Calif., assignors to California Research Corporation, San Francisco, Calif., a corporation of Delaware  
No Drawing. Filed Aug. 24, 1959, Ser. No. 835,391  
9 Claims. (Cl. 252—51.5)

9 Claims. (Cl. 252—51.5)

This invention pertains to lubricating oil compositions having incorporated therein metal-free detergents. These particular metal-free detergents are N-substituted alkenyl succinimides.

Alkenyl succinic anhydrides and numerous derivatives thereof are well known in the art. For example, alkenyl succinic anhydrides in which the alkenyl radical contains from 5 to 20 carbon atoms are taught as corrosion inhibitors in lubricating oil compositions. Also, products obtained by reacting such alkenyl succinic acid anhydrides with non-cyclic monamines are taught as ferrous corrosion inhibitors for lubricating oil compositions.

However, the above known alkenyl succinimides are not useful as detergents in lubricating oil compositions. In contrast thereto, the N-substituted polyamine alkenyl succinimides which are described herein are new compounds which are useful as detergents in lubricating oil compositions.

Present day internal combustion engines operate at high speeds and high compression ratios. When used in the so-called city stop-and-go driving, which includes the greater part of the driving condition for a large percentage of today's automobiles, the internal combustion engines do not reach the most efficient operating temperature. Under city driving conditions, large amounts of partial oxidation products are formed, and reach the crankcase of the engine by blowing past the piston rings. Most of these partial oxidation products are oil insoluble, tending to form deposits on the various operating parts of the engine, such as the pistons, piston rings, etc. For the purpose of preventing the deposition of these products on the various engine parts, it is necessary to incorporate detergents in the lubricating oil compositions, thus keeping these polymeric products highly dispersed in a condition unfavorable for deposition on metals.

For the most part, the various detergents which are added to crankcase oils to reduce this formation of sludges and varnishes are metal organic compounds, particularly those compounds wherein the metal is linked to an organic group through an oxygen atom. Although these metal-containing organic compounds have some effectiveness as detergents for dispersing the precursors of deposits within the oil itself rather than permitting them to form added deposits on the engine parts, they have the disadvantage of forming ash deposits in the engine. These ash deposits lower engine performance

2

by fouling spark plugs and valves, and contributing to preignition.

It is a particular object of this invention to provide lubricating oil compositions which are compounded with a metal-free detergent.

Therefore, in accordance with this invention, it has been discovered that lubricating oil compositions particularly useful for heavy duty service are obtained by incorporating N-alkylpiperazine monoalkenyl succinimides in oils of lubricating viscosity.

10 By the use of lubricating oil compositions containing  
the N-substituted alkenyl succinimides described herein,  
diesel and gasoline engine parts remain remarkably free  
15 of deposits and varnish, even under severe operating con-  
ditions.

The N-alkylpiperazine monoalkenyl succinimides are new compounds of the formula:



25 wherein R is a hydrocarbon radical having a molecular weight from about 400 to about 3000; that is, R is a hydrocarbon radical containing about 30 to about 200 carbon atoms; R' is a hydrocarbon radical containing from 1 to 3 carbon atoms; and R'' is hydrogen or a hydrocarbon radical containing from 1 to 3 carbon atoms.

These N-substituted alkenyl succinimides can be prepared by reacting maleic anhydride with an olefinic hydrocarbon followed by reacting the resulting alkenyl succinic anhydride with an N-( $\beta$ -aminoalkyl) piperazine. Such N-( $\beta$ -aminoalkyl) piperazines are well known.

Such N-( $\beta$ -aminoalkyl) piperazines are exemplified by N-methyl-N'-( $\beta$ -aminoethyl) piperazine, N-isopropyl-N'-( $\beta$ -aminoethyl) piperazine, N-( $\beta$ -aminoisopropyl) piperazine, etc.

The "R" radical of the above formula, that is, the alkenyl radical, is derived from an olefin containing from 2 to 5 carbon atoms. Thus, the alkenyl radical is obtained by polymerizing an olefin containing from 2 to 5 carbon atoms to form a hydrocarbon having a molecular weight ranging from about 400 to about 3000, more preferably, 900 to 1200. Such olefins are exemplified by ethylene, propylene, 1-butene, 2-butene, isobutene, and mixtures thereof. Since the methods of polymerizing the olefins to form polymers thereof is immaterial in the formation of the new compound described herein, any

50 of the numerous processes available can be used therefor.  
 The preparation of N-substituted monoalkenyl succinimides derived from amine derivatives of piperazine can be described generally by the following equations, using a polymer of isobutene as an example of the alkenyl radical; and N-( $\beta$ -aminoethyl) piperazine as an example of an N-(aminoalkyl) piperazine:





wherein  $n$  has a value of about 7 to about 50.

The above reaction between a polyolefin and maleic anhydride is an uncatalyzed addition reaction which should not be confused with a copolymerization reaction such as that obtained with a vinyl monomer and maleic anhydride. While the general reaction of an olefin and maleic anhydride is well known for olefins of low molecular weight (e.g., olefins of 18 carbon atoms), no previous work has been done with maleic anhydride and the high molecular weight olefins as described herein.

The reaction set forth and described by Equation I hereinabove can proceed in a mol ratio of the polyolefin to the maleic anhydride of 1:1 to 1:10, preferably from 1:1 to 1:5. The reaction temperature can vary from 300° F. to 450° F. Because of the greater yield of products obtained thereby, it is preferred to use the high range of temperatures (e.g., 375° to 450° F.).

In the second step of the reaction as exemplified by Equation II hereinabove, the yield of the imide is extremely high even though the reactants are used in equal molar ratios.

The reaction described by Equation II hereinabove can be made at 220° F. to 500° F., preferably from 300° F. to 400° F. The alkenyl succinic anhydride and the N-alkylaminopiperazines are reacted in about equal molar quantities.

Since the reaction between the polyolefin and maleic anhydride may not go to completion, the resulting alkenyl succinic anhydride may contain some unreacted polyolefin. As it may not be desirable to separate out this unreacted polyolefin at this stage, the resulting imide formed by reaction of the alkenyl succinic anhydride and the diamine will contain this polyolefin as an impurity which can be a diluent in the formation of lubricating oil compositions. However, if it is so desired, this unreacted polyolefin can be removed by precipitation, for example, by acetone or methanol from a hydrocarbon solution.

Lubricating oils which can be used as base oils include a wide variety of lubricating oils, such as naphthenic base, paraffin base, and mixed base lubricating oils, other hydrocarbon lubricants, e.g., lubricating oils derived from coal products, and synthetic oils, e.g., alkylene polymers (such as polymers of propylene, butylene, etc., and the mixtures thereof), alkylene oxide-type polymers (e.g., propylene oxide polymers) and derivatives, including alkylene oxide polymers prepared by polymerizing the alkylene oxide in the presence of water or alcohols, e.g., ethyl alcohol, dicarboxylic acid esters (such as those which are prepared by esterifying such dicarboxylic acids as adipic acid, azelaic acid, suberic acid, sebacic acid, alkanoic acid, succinic acid, fumaric acid, maleic acid, etc., with alcohols such as butyl alcohol, hexyl alcohol, 2-ethyl hexyl alcohol, dodecyl alcohol, etc.), liquid esters of acids of phosphorus, alkyl benzenes (e.g., monoalkyl benzene such as dodecyl benzene, tetradecyl benzene, etc., and dialkyl benzenes (e.g., n-nonyl 2-ethyl hexyl benzene); polyphenyls (e.g., biphenyls and terphenyls), alkyl biphenyl ethers, polymers of silicon (e.g., tetraethyl silicate, tetraisopropyl silicates, tetra-(4-methyl-2-tetraethyl) silicate, hexyl (4-methyl-2-pentoxy) disiloxane, poly(methyl siloxane, poly(methylphenyl) siloxane, etc. Synthetic

oils of the alkylene oxide-type polymers which may be used include those exemplified by the alkylene oxide polymers.

The above base oils may be used individually or in combinations thereof, wherever miscible or wherever made so by the use of mutual solvents.

The above-described alkenyl succinimides of this invention can be used in oils of lubricating viscosity in amounts of 0.1% to 80%, by weight, preferably 0.25% to 5%, by weight.

The preparation of N-alkylpiperazine alkenyl succinimides is illustrated in the following examples.

#### EXAMPLE I.—PREPARATION OF POLYBUTENYL SUCCINIC ANHYDRIDE

A mixture of 1000 grams (1 mol) of a polybutene having a molecular weight of about 1000 and 98 grams (1 mol) of maleic anhydride was heated at 410° F. in a nitrogen atmosphere with agitation for a period of 24 hours. The reaction mixture was cooled to 150° F. and 700 cc. of hexane added; after which the mixture was filtered under vacuum. After vacuum distillation to remove the hexane from the filtrate, the product was maintained at 350° F. at an absolute pressure of 10 mm. Hg for one hour to remove traces of maleic anhydride. The crude polybutenyl succinic anhydride thus prepared had a saponification number of 79.

#### EXAMPLE II.—PREPARATION OF N-ETHYLPIPERAZINE POLYBUTENYL SUCCINIMIDE ANHYDRIDE

A mixture of 18 grams (0.14 mol) of N-( $\beta$ -aminoethyl) piperazine and 200 grams (0.127 mol) of the polybutenyl succinic anhydride of Example I hereinabove was blended with agitation in a nitrogen atmosphere. The mixture was heated at 500° F. for one hour, after which the absolute pressure was reduced to about 200 mm. Hg to facilitate the removal of water and unreacted piperazine. The reaction mixture was then allowed to reach room temperature at this reduced pressure. The reaction product contained 2.59% nitrogen (theory=2.67%). Infra-red analysis showed that the reaction product was an imide containing a polybutene side chain.

Table I hereinbelow presents data obtained with lubricating oil compositions containing N-alkylpiperazine monoalkenyl succinimides.

The tests were made in a Caterpillar L-1 engine according to Mil-L-2104 conditions for a period of 120 hours as described in the Coordinating Research Council Handbook, January 1946.

The "PD Nos." refer to the piston discoloration rating. After the engine test, the three piston lands are examined visually. To a piston skirt which is completely black is assigned a PD number of 800; to one which is completely clean, a PD number of 0; to those intermediate between completely black and completely clean are assigned PD numbers intermediate in proportion to the extent and degree of darkening.

The "GD Nos." refer to the percentage deposits in the piston ring grooves; and 0 evaluation being a clean groove; and a number of 100 being a groove full of deposits.

The base oils were California SAE 30 base oils.

The monoalkenyl succinimide used was an N-substituted succinimide derived from N-( $\beta$ -aminoethyl) piperazine, wherein the alkenyl radical had a molecular weight of about 1000, which alkenyl radical was a polymer of isobutene.

The dithiophosphate was a zinc salt of a mixed dialkyl dithiophosphate wherein one of the alkyl radicals contained 4 carbon atoms and the other alkyl radical contained 5 carbon atoms. The dithiophosphate was present in the lubricating oil compositions in an amount of 12 millimols per kilogram (i.e., 12 mM./kg.) of finished product.

Table I

| Additive                     | A             | B        | C        |
|------------------------------|---------------|----------|----------|
| Succinimide*, weight percent | 0.0           | 1.0      | 1.0      |
| Dithiophosphate, mM./kg.     | 0.0           | 0.0      | 12       |
| Test Results:                |               |          |          |
| GD No.                       | 39            | 1        | 0.3      |
| PD No.                       | 800, 800, 800 | 25, 0, 5 | 10, 0, 0 |

Table II hereinbelow presents data obtained in an FL-2 test, using a 6-cylinder Chevrolet engine operating at 2500 r.p.m. for a period of 40 hours, which test is fully described in a Coordinating Research Council bulletin titled "Research Technique for the Determination of the Effects of Fuels and Lubricants on the Formation of Deposits During Moderate Temperature Operation" (1948).

The piston varnish rating is a visual observation of the amount of varnish on a piston skirt, with "10" being the maximum rating for a perfectly clean piston and a "0" being the rating of a piston fully covered with black varnish. This piston varnish rating correlates with road performance in automobiles.

The base oil was an SAE 30 base oil.



The succinimide and the dithiophosphate were the same as those described for Table I hereinabove.

Table II

| Additive                            | D   | E        |
|-------------------------------------|-----|----------|
| Succinimide, Wt. percent            | 0.6 | 1.0      |
| Dithiophosphate mM./kg.             | 13  | 13       |
| Test results: Piston varnish rating | 5.7 | 6.9, 7.8 |

It is readily seen from the data set forth hereinabove in Tables I and II that lubricating oil compositions containing the N-alkylpiperazine alkenyl succinimides as described herein are superior as lubricating oil compositions for the lubricating of internal combustion engines.

In addition to the dithiophosphate described hereinabove, lubricating oil compositions containing the N-substituted alkenyl succinimides of N-alkylpiperazine of this invention may also contain other detergents, viscosity index improving agents, rust inhibitors, oiliness agents, grease thickening agents, etc.

We claim:

1. A lubricating oil composition consisting essentially of an oil of lubricating viscosity and from 0.1% to 80%, by weight, of an N-alkylpiperazine monoalkenyl succinimide of the formula:



wherein R is a hydrocarbon radical having a molecular weight from about 400 to about 3000, and R' is a hydrocarbon radical containing from 1 to 3 carbon atoms.

2. A lubricating oil composition consisting essentially of an oil of lubricating viscosity and from 0.1% to 80%, by weight, of an N-alkylpiperazine monoalkenyl succinimide of the formula:



wherein R is a hydrocarbon radical having a molecular weight from about 900 to about 1200, and R' is a hydrocarbon radical containing from 1 to 3 carbon atoms.

3. A lubricating oil composition comprising a major proportion of an oil of lubricating viscosity and from 0.25% to 5%, by weight, of an N-alkylpiperazine monoalkenyl succinimide of the formula:



wherein R is a hydrocarbon radical having a molecular weight from about 900 to about 1200, and R' is a hydrocarbon radical containing from 1 to 3 carbon atoms, and R'' is selected from the group consisting of hydrogen and hydrocarbon radicals containing from 1 to 3 carbon atoms.

4. A lubricating oil composition comprising a major proportion of a petroleum lubricating oil and from 0.25% to 5%, by weight, of an N-substituted monoalkenyl succinimide of the formula:



wherein n has a value of about 7 to about 50.

5. A lubricating oil composition comprising a major proportion of an oil of lubricating viscosity and a minor proportion, in an amount sufficient to impart detergency to said oil, of an N-alkylpiperazine monoalkenyl succinimide of the formula:



wherein R is a hydrocarbon radical having a molecular weight from about 400 to about 3,000, R' is a hydrocarbon radical containing from one to three carbon atoms, and R'' is selected from the group consisting of hydrogen and hydrocarbon radicals containing from 1 to 3 carbon atoms.

6. A lubricating oil composition comprising a major proportion of an oil of lubricating viscosity and a minor proportion, an amount sufficient to impart detergency to said oil, of an N-alkylpiperazine monoalkenyl succinimide of the formula:



wherein R is a hydrocarbon radical containing from about 30 to about 200 carbon atoms formed by polymerizing

olefins containing from 2 to 5 carbon atoms, and R' is a hydrocarbon radical containing from 1 to 3 carbon atoms.

7. A lubricating oil composition consisting essentially of an oil of lubricating viscosity and from about 0.1% to about 80%, by weight, of an N-alkylpiperazine mono-alkenyl succinimide of the formula:



wherein R is an alkynyl radical containing from 30 to 200 carbon atoms and which is a polymer of an olefin containing from 2 to 5 carbon atoms, and R' is an alkyl radical containing from 1 to 3 carbon atoms.

8. A lubricating oil composition comprising a major

proportion of an oil of lubricating viscosity and from 0.25% to 5%, by weight, of an N-alkylpiperazine mono-alkenyl succinimide of the formula:

5



1

wherein R is an alkenyl radical containing from 30 to 200 carbon atoms and is a polymer of an olefin containing from 2 to 5 carbon atoms, and R' is an alkyl radical containing from 1 to 3 carbon atoms.

9. A lubricating oil composition consisting essentially of a petroleum lubricating oil, and from 0.1% to 80%, by weight, of an N-substituted monoalkenyl succinimide of the formula:



wherein  $n$  has a value of about 7 to about 50.

References Cited in the file of this patent

UNITED STATES PATENTS

- |           |                    |               |
|-----------|--------------------|---------------|
| 2,490,744 | Trigg et al. ----- | Dec. 6, 1949  |
| 2,604,451 | Rocchini -----     | July 22, 1952 |
| 2,638,450 | White et al. ----- | May 12, 1952  |

UNITED STATES PATENT OFFICE  
CERTIFICATION OF CORRECTION

Patent No. 3,024,195

March 6, 1962

Alan Y. Drummond et al.

It is hereby certified that error appears in the above numbered patent requiring correction and that the said Letters Patent should read as corrected below.

Columns 1 and 2, bottom of the page, the front end portion of the reactant and the reaction product of the equations, and the top of column 3, two occurrences, should appear as shown below instead of as in the patent:



column 2, lines 18 to 24, column 5, lines 69 to 75, column 6, lines 8 to 13, lines 21 to 27, lines 49 to 55, lines 67 to 73, column 7, lines 7 to 13, and column 8, lines 4 to 9, the left-hand portion of the formula, each occurrence, should appear as shown below instead of as in the patent:



Signed and sealed this 17th day of July 1962.

SEAL)

Attest:

ERNEST W. SWIDER

Attesting Officer

DAVID L. LADD

Commissioner of Patents